

July 21, 1936.

J. M. YOUNG

2,048,478

BOTTLE BREAKING DEVICE

Filed Sept. 26, 1934

2 Sheets-Sheet 2

Fig. 5



Fig. 6



Fig. 7



INVENTOR  
John M. Young  
Drawn by D. Shombrugh  
ATTORNEY

## UNITED STATES PATENT OFFICE

2,048,478

## BOTTLE BREAKING DEVICE

John M. Young, Brooklyn, N. Y., assignor to  
Rebecca R. Young, Brooklyn, N. Y.

Application September 26, 1934, Serial No. 745,586

7 Claims. (Cl. 49—52)

The present invention relates to a bottle breaking device and has particular reference to a simple, manually operated bottle crusher in the use of which a breaking action is applied in a concentrated zone on the bottle so that it is rendered unfit for use but is not broken to that extent where it would present a hazard in subsequent handling during its discard.

At the present time bottles after being emptied of the legitimate liquor that they contained have come into the hands of unscrupulous persons, bootleggers, who have reused them for spurious and imitation liquors passing them off as the genuine product in accordance with the label designation or other insignia on the bottle, thus deceiving the public and depriving both State and Federal Governments of revenue. This practice has been accentuated since the repeal of the Federal Prohibition Law, that is, the Eighteenth Amendment to the Constitution.

An awakened public becoming aware of such practices has found it desirable to break the bottles to prevent their reuse, but it is both difficult and dangerous for the average person to break a bottle owing to the hazard of flying glass and the hazard of the subsequent handling of the broken parts of the bottle.

An object of the present invention is the provision of a bottle breaking device which breaks out only a small section from that part of a bottle which is used directly in the sealing of its enclosed contents, in other words the cork part or cap part of the neck of the bottle, so that it cannot be used again, its sealing zones having been destroyed. The breaking out of this section is so controlled and so concentrated that danger of flying glass is obviated and yet the bottle, after breaking may be handled without cutting hazard.

A further object is the provision of a bottle breaking device with a support for the bottle neck and a breaking element so arranged and so operated as to confine the lines of breaking strains to a single, relatively small place of application at the rim on the neck by means of which only the desired minimum area is affected.

Another object of the invention is the provision of such a device wherein concentration and application of a limited force of impact is brought to bear on the bottle being broken.

Still another object is the provision of a bottle breaking device of the character described wherein a confined and accumulating pressure or breaking force is applied on the neck of the bottle at a single zone of rupture.

Yet another object is the provision of a collecting element associated with the bottle crusher which receives and retains the broken glass pieces resulting from the breaking action.

Numerous other objects and advantages of the invention will be apparent as it is better understood from the following description, which, taken in connection with the accompanying drawings, discloses a preferred embodiment thereof.

Referring to the drawings:

Figs. 1 and 2 illustrate a preferred embodiment of the present invention and show an impact type of bottle crusher, Fig. 1 being a perspective view of the bottle crushing device particularly showing the side of the device that is applied to the bottle to be broken, while Fig. 2 is a longitudinal section of the same showing it on the bottle with its parts in the position assumed at the conclusion of the breaking action.

Fig. 3 is a perspective view of a modified form of the invention illustrating a pressure applying type of bottle crusher:

Fig. 4 is a fragmentary side elevation of the upper or neck end of a bottle which has been subjected to the action of the bottle crusher and showing the restricted nature of the part broken out;

Fig. 5 is another modified form of bottle crushing device being an adaptation of the impact type illustrated in Figs. 1 and 2 and being further provided with bottle retaining and collecting features;

Fig. 6 is a side elevation partially in section of still a different form of bottle breaking device of the pressure type, the position of the bottle neck to be broken being shown in dot-and-dash lines; and

Fig. 7 is a fragmentary sectional view taken substantially along the line 7—7 in Fig. 6 showing the bottle neck wall engaged for crushing.

In the disclosure of the bottle crusher illustrated in Figs. 1 and 2 there is shown a body member 11 formed generally as a block which is cut away at 12 to provide a receiving part for the neck of a bottle to be broken. In positioning the crusher for use, a wall 13 formed in the cut-away section 12 is placed on the upper end of the bottle neck designated generally by the numeral 15 and in this position a support block 16 contacts the bottle neck on one side.

Block 16 is formed with an inner cylindrical wall 17 which merges at its terminal ends in walls or projections 18. These projections directly engage the bottle neck 15 and center it against the wall 13. The block 16 is secured to

ing or breaking lug 73 which is formed with a tapered front or striking face 74.

At the time the bottle is placed in position for breaking the lug 73 is inside of the bottle neck, being held in its non-operated position against a retaining plate 75 which is set into the upper surface of the body 61 and is secured at 76 to the under surface of the block 65. A spring 77 is preferably mounted on the bar 71 and is located outside of the crusher body, being confined between washers 78 which are also mounted on the bar. The outer washer bears against a pin 79 carried in the bar.

In this initial bottle receiving position of the device, that is, with the projection lug 73 of the bar 71 against the plate 75, the spring 77 is in its limited expanded position holding the sliding bar 71 out or toward the right.

The breaking of the bottle and the forming of a fracture 35 within the bottle neck is effected by striking the outer end of the bar 71 with any suitable device as by a hammer block 81. This creates a crushing force or impact which is applied outwardly against the confined parts of the bottle neck supported exteriorly by the support block 68 and under striking force of the lug 73. For convenience the hammer block may be connected with the device by a flexible chain 82.

A retaining chamber 85 is formed in the base of the body member 61 and at the top this chamber communicates with a vertical bore 86 formed in the body, the lug 73 and the front end of the bar 71 having movement within this opening. In the crushing action broken bits of glass 81, which are broken out of the fracture 35 in the bottle wall, fall through the opening 86 and drop into the chamber 85. A sliding door 88 may be used to effect a closure for this chamber, this door preferably having sliding movement within suitable guideways 89 formed in a recessed bottom of the body 61.

The chamber 85 is adequate to collect and retain the broken bits of glass from several bottles and thus acts as a reservoir so that the broken glass pieces are retained in the chamber. To empty the chamber it is merely necessary to withdraw the slide 88 (Fig. 5 showing an intermediate step in the withdrawing action) and the bottom of the chamber is opened for the discharge of the broken bits. In this form of crusher all glass is caught and there will not be any flying glass hazard.

In the modified form illustrated in Fig. 6 the bottle crusher is similar in general principle to a pair of pliers. Pivotal handle parts 91, 92 are associated for pivotal movement relative to each other. A pivot bolt 93 passes loosely through the wall of the member 91 and engages within the member 92 for this purpose. The part 92 is formed with a bottle neck enclosing section or body 95 which preferably extends down in a depending skirt 96 inside of which is a bottle neck receiving chamber 97.

The chamber is open at the bottom and along one side, the skirt 96 extending back into projecting spaced walls 98 adjacent the open side. A central post 99 is preferably carried in the body 95 and a projecting end 101 extends down into the top part of the chamber 97. The post 99 constitutes the stationary element or crushing lug of the device. The forward end of the handle member 91 below its pivot connection 93 is formed in a curved section 102 the terminal edge of which is rounded off in a nose 103, this constituting the movable crushing element.

In use this form of bottle crusher is placed over the bottle to be broken with the upper end of its neck within the chamber 97. The post 101 thereupon extends down inside of the neck. Squeezing of the handle parts 91, 92 forces the rounded nose 103 to move into the wall of the bottle neck from the outside. The force exerted on the bottle at the nose is applied directly opposite to the supporting forces provided by the post end 101. A recess 104 is formed in this end of the post on the side facing the nose 103 so that there is provided a three-point support (Fig. 7) on the engaged bottle neck for the crushing action. This three-point engagement effects a restricted breaking action by setting up breaking strains in the bottle neck 15 which break the bottle wall and produce a fracture as shown at 35 in Fig. 4. The broken bits of glass are mostly forced into the interior of the bottle and the skirt 96 further acts as a shield to prevent any flying of the glass.

It is thought that the invention and many of its attendant advantages will be understood from the foregoing description, and it will be apparent that various changes may be made in the form, construction and arrangement of the parts without departing from the spirit and scope of the invention or sacrificing all of its material advantages, the form hereinbefore described being merely a preferred embodiment thereof.

I claim:

1. A bottle breaking device comprising a support for the outside rim of the neck of a bottle to be broken, a movable instrumentality associated with said support and disposed transversely of the bottle neck rim edge and means movable with said instrumentality and cooperating with said support and movable toward it and engageable inside of said bottle neck for forcing a part of the confined neck wall outwardly to break the same.

2. A bottle breaking device, comprising a body member for engaging the rim edge of the neck of a bottle to be broken, a supporting wall carried by said body member for engaging the side wall of a restricted part of the bottle neck, a movable instrumentality slidably mounted in said body member, and a breaking member carried by said instrumentality and adapted for passage through the supported bottle part adjacent said supporting wall for breaking out a restricted rim portion thereof.

3. A bottle breaking device, comprising a body member adapted to be disposed over the open end of a bottle to be broken and engageable with the rim edge thereof, a supporting wall associated with said body member for engaging a restricted part of the bottle on a side thereof, an instrumentality movable relative to said supporting wall and transversely of the bottle mouth, and means applicable through said instrumentality and during movement of the same to apply a breaking force against the bottle neck and at the engaged rim to break out a restricted portion thereof.

4. A bottle breaking device, comprising a body member for receiving the neck of a bottle to be broken and for holding the bottle inverted and resting on its rim edge, a side support mounted on said body member and adapted to engage the side of the bottle neck, and breaking means movable transversely of the bottle neck while engaged with said support for applying a breaking force adjacent the supported parts of said neck to break out a restricted rim portion of the same, said body member having a receiving chamber which is in open communication with the bottle 75

neck edge and into which the broken parts of said neck are collected as the same are removed by said breaking means.

5. A bottle breaking device, comprising a body member adapted to be placed on top of a bottle to be broken and in engagement with the rim edge of its neck, a supporting wall carried by said body member for engaging a restricted part of the side of the bottle neck, and a breaking member carried in said body member and movable transversely of the said bottle neck and toward said supporting wall to first press the engaged bottle part against said supporting wall and then to completely pass through the engaged part for breaking away a restricted rim portion only of said neck and leaving a substantial part of the rim surrounding the bottle mouth.

6. A bottle breaking device, comprising a body member for engaging the rim edge of the neck of a bottle to be broken, a supporting wall carried by said body member for engaging a restricted part of the side wall of the bottle neck, a movable instrumentality slidably mounted in said body member and having a face movable across and in contact with the rim edge of said engaged bottle, a breaking member carried by said instrumentality and adapted for passage through the

supported bottle neck part adjacent said supporting wall when said sliding instrumentality is struck by a hammer unit flexibly secured to said body member, and means for returning said instrumentality into normal position after such a 5 striking blow.

7. A bottle breaking device, comprising a body member for engaging the rim edge of the neck of a bottle to be broken, a supporting wall carried by said body member for engaging a re- 10 stricted part of the side wall of the bottle neck, a movable instrumentality and insertable in said bottle neck slidably mounted in said body member, a breaking member carried by said instrumentality and adapted for breaking outwardly 15 through the supported bottle neck part adjacent said supporting wall when said sliding instrumentality is moved under the impact of a hammer unit flexibly secured to said body member, means for returning said instrumentality into 20 normal position after its movement, and a receiving chamber formed in said body member and having open communication with the bottle neck when engaged by said supporting wall for collecting the broken parts of said bottle which 25 are removed by said breaking member.

JOHN M. YOUNG.

## UNITED STATES PATENT OFFICE

2,048,479

## LUBRICANT FOR FREE-WHEELING

Elmer Wade Adams and George Mervin McNulty,  
Hammond, Ind., assignors to Standard Oil  
Company, Chicago, Ill., a corporation of  
Indiana

No Drawing. Application February 3, 1933,  
Serial No. 655,000

11 Claims. (Cl. 87-9)

This invention relates to a new lubricant and it pertains more particularly to a lubricant for use with free-wheel drives or free-wheel clutches and will be referred to hereinafter as a free-wheel lubricant.

For free-wheel clutches to operate successfully under all temperature conditions, great care must be exercised in the selection of the lubricant. It is essential to employ a lubricant having a low viscosity temperature coefficient as indicated by a high viscosity index. If lubricants with low viscosity indices are used, the free-wheel clutch will not operate successfully at low temperatures generally encountered during the winter months.

15 The significance of the viscosity index is described in the Industrial and Engineering Chemistry, by Dean and Davis, volume 36, page 618, 1929.

The operation of free-wheeling devices is greatly influenced by the viscosity of the lubricant used therein because a slight change in viscosity of the oil will greatly affect the operation of said devices. As stated above, the oils used for lubrication in these free-wheeling devices must possess a low viscosity temperature coefficient, that is, the change in viscosity of the oil with temperature fluctuations must be a minimum. The inherent resistance of an oil to change in viscosity with temperature fluctuations can be expressed by the viscosity index of the oil. For example, the viscosity of Pennsylvania oils which are highly paraffinic, suffers relatively small changes at different seasonal temperatures and consequently the viscosity indices of such oils are high. By definition, oils of this type have been assigned a viscosity index of 100. On the other hand, the viscosity of Mid-Continent oils, which are highly naphthenic, undergoes a greater change at different seasonal temperatures and consequently the viscosity indices of Mid-Continent oils are relatively low, ranging from about 40 to 70. This range of viscosity indices is characteristic of the mixed base oils. Coastal oils have viscosity indices of about zero and certain California oils have lower viscosity indices.

45 The pour point of the lubricant used in free-wheeling devices must be low enough so that the clutch will not become inoperative during the winter months. At low temperatures some oils used for free-wheeling tend to solidify and become very viscous. Such an oil will not permit the clutch to operate as designed and cause grabbing and slipping of the clutch. At the same time, the heavy bearing loads carried by the moving parts of these devices require the use of a fairly heavy lubricant under ordinary conditions,

making it undesirable to obtain cold weather fluidity by selecting a light oil.

The object of our invention is to provide a lubricating oil compounded from mixed base oils or Pennsylvania oils, which are suitable for use in free wheeling devices, and which have a high viscosity index.

Another object is to provide such oils from mixed base lubricating distillates.

A further object of our invention is to provide lubricating oils suitable for use in free wheeling devices and which have low pour points.

We have found that a composition comprising a mineral oil and sulfurized cottonseed oil can be successfully used in free wheeling clutches and related devices wherein oils of high viscosity indices and low pour points are needed. These lubricants are prepared by blending from 10 to 15 parts of sulfurized cottonseed oil with about 90 to 85 parts of a mixed base oil to give a resulting composition containing from 0.5 to 3% of sulfur. However, the preferred total sulfur content of the composition should be from 1 to 2%. The viscosity of the mixed base oils used in preparing our free wheeling lubricant may vary considerably depending on whether a light, medium or heavy type of oil is desired. Generally the viscosity of the base oil lies above 200 seconds Saybolt at 100° F. Other sulfurized vegetable oils of substantially the same chemical composition as sulfurized cottonseed oil may also be used.

The sulfurized cotton seed oil is prepared by adding 11 to 25% of sulfur to the cottonseed oil and heating the mixture at a temperature ranging from 300 to 400° F. for 15 to 20 hours. For example, sulfurized cottonseed oil herein described was prepared by adding 12% of sulfur to cottonseed oil and heating the mixture at a temperature of about 340-360° F. for 18 to 20 hours. The oil may then be filtered or passed through a fine mesh screen. The resulting product had a sulfur content of 8.5% and a pour point of about plus 40° F. The sulfur content of the sulfurized cottonseed oil may suitably range from 5 to 15% and, if desired, 100% sulfurized cottonseed oil may be used.

Our new lubricating oil is prepared by dissolving the sulfurized cottonseed oil in a mineral oil having a sufficiently high viscosity index to give a blend of the desired properties. We prefer to use a mixed base oil having a viscosity index ranging from 50 to 80 but other oils may be used, such as Coastal oils and Pennsylvania oils which have lower and higher viscosity indices, respectively. The sulfurized cottonseed oil may

be added to the oil in varying proportions, however, we have found that a total sulfur content of about 1 to 3% is satisfactory for most purposes. Larger percentages of sulfur may be present in the final composition if corrosion is not a factor to be considered in the use of the oil. Generally about 11 to 25 parts of the above sulfurized cottonseed oil, containing 8.5% of sulfur, is mixed with 75 to 100 parts of the mixed-base oil.

In order to illustrate the unique properties of our new composition, we have compared it with a blend of sulfurized lard oil and mixed base lubricating oil. The following tables disclose the properties of the sulfurized cottonseed oil and sulfurized lard oil, and also the properties of the blends of these sulfurized oils with mineral oils:

Table I

|                       | Properties of:            |                     |
|-----------------------|---------------------------|---------------------|
|                       | Sulfurized cottonseed oil | Sulfurized lard oil |
| Viscosity at 210° F.  | 422                       | 170                 |
| Viscosity at 130° F.  | 2102                      |                     |
| Pour.                 | +40° F.                   | 65° F.              |
| Acidity (mg. KOH/gm.) | 6.80                      | 35.00               |
| Sulfur.               | 8.51                      | 6.51                |

Table II

| Examples                    | Parts used to give 1% of sulfur in blend | Viscosity index of the mineral oil before blending | Properties of the blend or free-wheel lubricant |            |                 |
|-----------------------------|------------------------------------------|----------------------------------------------------|-------------------------------------------------|------------|-----------------|
|                             |                                          |                                                    | Vis. at 100° F.                                 | Pour point | Viscosity index |
| A Sulfurized cottonseed oil | 11                                       | 55                                                 | 215                                             | -10° F.    | 116             |
| Sulfurized lard oil         | 14                                       | 55                                                 | 213                                             | 0° F.      | 92              |
| B Sulfurized cottonseed oil | 11                                       | 72                                                 | 980                                             | -5° F.     |                 |
| Sulfurized lard oil         | 14                                       | 72                                                 | 853                                             | +10        |                 |
| C Sulfurized cottonseed oil | 11                                       | 67                                                 | 2000                                            | +20        | 103             |
| Sulfurized lard oil         | 14                                       | 67                                                 | 2522                                            | +30        | 87              |

From the above data it will be observed that both compositions contain enough of the sulfurized animal or vegetable oil to give a total sulfur content of 1%. The compositions containing sulfurized cottonseed oil have a lower pour point than the compositions containing the sulfurized lard oil, also the former have a higher viscosity index than the latter. In Example A it will be noted that the composition containing sulfurized cottonseed oil has a pour point of -10° F. and a viscosity index of 116, whereas the composition containing sulfurized lard oil has a pour point of 0° F. and viscosity index of 92.

The sulfurized cottonseed oil is particularly suitable for making lubricants for free-wheeling devices, because it greatly increases the viscosity index of the base stock. In Example A of Table II it will be observed that the viscosity index of the base stock was 55, whereas the blend has a viscosity index of 116. In other words, the sulfurized cottonseed oils tend to prevent the oils from changing in viscosity at different temperatures. It will also be observed that the free-wheeling lubricant described in Example A has a higher viscosity index than Pennsylvania oils.

The sulfurized cottonseed oil blends have proven to be very successful for lubricating free-wheeling devices wherein great operating stresses are applied to a sensitive mechanism.

With some lubricants it is necessary to drive a car for five or ten minutes with the free-wheel

unit locked so that the lubricant may be whipped up sufficiently to allow the clutch roller to function properly. This difficulty is not encountered with our sulfurized cottonseed oil lubricant. Also our lubricant greatly reduces the noise that generally accompanies the operation of most free-wheeling devices.

We have described our invention with reference to specific oils and proportions of oil, however, it is not intended that such disclosure be considered as a limitation upon the scope of our invention except insofar as included in the appended claims.

We claim:

1. A free-wheel lubricant consisting of a blend of a mixed base oil and sulfurized cottonseed oil, the sulfur content of said lubricant ranging from 0.5 to 3%.

2. A free-wheel lubricant having a viscosity index greater than 100 which consists of a blend of a mixed base mineral oil and sulfurized cottonseed oil, the sulfur content of said lubricant not exceeding 3%.

3. A free-wheel lubricant having a viscosity index ranging from 100 to 116 and a pour point below 0° F. which consists of a blend of a mixed base mineral oil having a Saybolt viscosity above 200 at 100° F. and sulfurized cottonseed oil.

4. A free-wheel lubricant which consists of a blend of a mixed base mineral oil having a viscosity above 200 seconds Saybolt at 100° F. and sulfurized cottonseed oil, the sulfur content of said lubricant not exceeding 3%.

5. A free-wheel lubricant having a viscosity index above 100 which consists of from 85 to 90 parts of a mixed base mineral oil and from 10 to 15 parts of sulfurized cottonseed oil.

6. A free-wheel lubricant having a viscosity index above 100 and a pour point below 0° F. which consists of a blend of a mineral oil and sulfurized cottonseed oil, the total sulfur content of the lubricant ranging from 0.5 to 3%.

7. A free-wheel lubricant having a viscosity index above 100 and a pour point below 0° F. which comprises substantially entirely a blend of a mixed base oil having a Saybolt viscosity above 200 at 100° F. and a viscosity index below 100, and sulfurized cottonseed oil, the total sulfur content of the lubricant not exceeding 3%.

8. A free-wheel lubricant having a viscosity index above 100 and a pour point below 0° F. which consists of a blend of a mineral oil having a viscosity between 215 and 980 seconds Saybolt at 100° F. and sulfurized cottonseed oil, the total sulfur content of the lubricant ranging from 0.5 to 3%.

9. The method of preparing a free-wheel lubricant having a viscosity index above 100 and a pour point below 0° F. which comprises blending 85 to 90 parts of a mineral oil having a